

## [54] COGENERATION PROCESS FOR PRODUCTION OF ENERGY AND IRON MATERIALS

[75] Inventor: John M. Lehto, Cokato, Minn.

[73] Assignee: Northern States Power Company, Minneapolis, Minn.

[21] Appl. No.: 423,615

[22] Filed: Oct. 16, 1989

## Related U.S. Application Data

[63] Continuation of Ser. No. 91,427, Aug. 31, 1987, abandoned.

[51] Int. Cl.<sup>5</sup> ..... C21B 11/02

[52] U.S. Cl. ..... 75/499; 75/958; 208/426; 208/427

[58] Field of Search ..... 208/427, 426; 75/500, 75/499, 501, 502, 958; 266/160

## [56] References Cited

## U.S. PATENT DOCUMENTS

|           |         |                  |       |          |
|-----------|---------|------------------|-------|----------|
| 2,034,071 | 3/1936  | Wickland         | ..... | 266/24   |
| 3,479,021 | 11/1969 | Escher           | ..... | 266/31   |
| 3,617,042 | 11/1971 | Nakagawa         | ..... | 266/34 R |
| 3,801,305 | 4/1974  | Nilles et al.    | ..... | 75/60    |
| 3,918,958 | 11/1975 | Heitmann         | ..... | 414/786  |
| 4,008,054 | 2/1977  | Clancy et al.    | ..... | 208/427  |
| 4,025,059 | 5/1977  | Steinmetz et al. | ..... | 266/215  |
| 4,057,231 | 11/1977 | Chazé            | ..... | 266/219  |
| 4,309,024 | 1/1982  | Lillybeck et al. | ..... | 266/900  |
| 4,495,054 | 1/1985  | Claflin          | ..... | 75/29    |
| 4,504,043 | 3/1985  | Yamaoka et al.   | ..... | 266/218  |
| 4,511,372 | 4/1985  | Axelson          | ..... | 75/501   |
| 4,753,677 | 6/1988  | Rachner          | ..... | 75/59.18 |
| 4,874,427 | 10/1989 | Hamada et al.    | ..... | 266/160  |

## FOREIGN PATENT DOCUMENTS

|         |        |                      |       |       |
|---------|--------|----------------------|-------|-------|
| 44669   | 1/1982 | European Pat. Off.   | ..... | 75/3  |
| 139310  | 5/1985 | European Pat. Off.   | ..... |       |
| 1583974 | 9/1970 | Fed. Rep. of Germany | ..... |       |
| 3345107 | 9/1984 | Fed. Rep. of Germany | ..... |       |
| 3510787 | 9/1986 | Fed. Rep. of Germany | ..... | 75/29 |
| 3523487 | 1/1987 | Fed. Rep. of Germany | ..... |       |
| 2011575 | 3/1970 | France               | ..... |       |
| 2003496 | 3/1977 | United Kingdom       | ..... |       |

## OTHER PUBLICATIONS

*Steel & Coal*, 185, 304 at p. 305 (Aug. 17, 1962).*Energy Progress*, 2, 121 (1982).*DOE Report*, "Development of an Advanced, Continuous Mild Gasification Process for the Production of Co-Products—Industrial Market Assessment of the Products of Mild Gasification", J. E. Sinor et al., Jan. 1988.*DOE Report*, "Development of an Advanced, Continuous Mild Gasification Process for the Production of

(List continued on next page.)

*Primary Examiner*—Melvyn J. Andrews  
*Attorney, Agent, or Firm*—Merchant, Gould, Smith, Edell, Welter & Schmidt

[57]

## ABSTRACT

A process and arrangement are provided for the efficient generation of energy from coal, while at the same time providing for a relatively inexpensive step in processing of iron or steel, and the extraction of valuable materials such as oils from coal. An advantage to the process is that relatively low quality coals can be utilized, since the coal is pretreated before any burning operation. Generally, the process involves three interacting stages. In the First Stage, a coal liquefaction/pyrolysis procedure is utilized to drive off volatiles, and form a very low volatile char. The volatiles can be collected and utilized as a valuable oil product, such as for diesel fuel or the like. The char material is preferably pelletized and utilized as a reductant, in a Second Stage of iron reduction and melting. Preferably the iron reduction and melting operation is conducted in a cupola and the hot product gases are utilized directly and/or indirectly, to generate electricity in Stage Three, and to produce hot steam for use in driving certain portions of Stages One and Two.

6 Claims, 2 Drawing Sheets



OTHER PUBLICATIONS

Co-Products—Literature Survey Results", W. G. Willson et al., Jan. 1988.  
*Clean Coal Technologies*, 89, 9 (1989).  
Pellet Technology Corporation "Technology Overview," Mar. 1986.  
K. W. Lange, "Thermodynamics and Kinetics at High Temperature in Ladle Metallurgy," *Proceedings of the Second International Conference on Iron & Steel Technology and New Materials*, Oct. 7-9, 1986, Pohang, Republic of Korea, p. 43, Tables 5-6 at pp. 76-77.  
Klara et al., *Paper Presented at Alternate Energy '89, "Mild Gasification: A New Goal"* (published Apr. 1989).  
Suumberg et al., *Fuel*, 64, 1668 (1985).

Derbyshire et al., *Fuel*, 65, 1233 (1986).  
Derbyshire et al., *Fuel*, 66, 1741 (1987).  
Derbyshire et al., *EPRI Pub. No. GS-6219* (published Jan. 1989).  
*DOE Pub. No. DOE/FE-0115-11* (published Jan. 1989).  
"Costs of Synthetic Fuels in Relation to Oil Prices," a report prepared for the Subcommittee on Energy Development and Applications, 97th Congress, Mar. 1981.  
"Synthetic Fuel Technology Development in the United States," A Retrospective Assessment by M. Crow et al., (1988), (pp. ix, x, xi, 32, 33, 46, 47).  
"Gasification: Key to Chemicals from Coal" by J. S. Wilson et al., *Chemtech*, Feb. 1988.  
"Process Improvements in Direct Liquefaction of Coal," Technical Brief, 1989.

—  
FIG.





## COGENERATION PROCESS FOR PRODUCTION OF ENERGY AND IRON MATERIALS

This is a continuation of application Ser. No. 5 07/091,427, filed Aug. 31, 1987 now abandoned.

### FIELD OF THE INVENTION

The present invention relates to thermoelectric power generation. In particular, the invention concerns the generation of power, from coal. A cogeneration process is involved, whereby a coal fuel is treated in a liquefaction procedure or step, for removal of valuable oils and the like therefrom. The resultant low-volatiles char is then useable in an iron reduction and melting process. During the high temperature iron refining process, product gases are generated. The gases are used, directly and/or indirectly, to power turbines and generate electrical power. The overall process particularly concerns a system in which advantage is taken of the characteristics of each individual step or stage, to facilitate an overall relatively energy efficient process.

### BACKGROUND OF THE INVENTION

In recent decades achievement of efficient and relatively inexpensive electrical energy production has become a major concern. Of the various types of power plants, coal-burning plants have been particularly popular and widely used. The reasons for this include relative adaptability to a variety of locations and relatively wide availability of a comparatively inexpensive fuel.

A problem with conventional coal burning systems involves the general methodology of fuel use. In a typical system the coal is simply burned, with the waste discarded. This has generated two substantial concerns. First, coal fuels often include therein relatively useful organic fractions, which could be isolated and refined to useful oil products, such as diesel fuel or the like. Typically in conventional plants these fractions are merely burned, as an inexpensive fuel, along with the remainder of the coal. It is readily seen that this, arguably, is an inefficient utilization of the coal as a natural resource.

Secondly, conventional systems generally require a relatively high grade of fuel coal. For example, coal having a substantial amount of sodium therein is not readily utilizable, as it does not burn well. If such materials in the coal were first extracted therefrom, a lower grade coal could be effectively used as a fuel source.

Methods of coal liquefaction, i.e. the removal of volatile materials from coal, are well-known. Generally, however, such processes have not been practiced on coal to be utilized as a fuel for power generation. A major reason for this is that the resultant coal char has not been a desirable fuel. While such char has a significant energy content, it generally does not burn well and cleanly in conventional boilers. Thus, the use of char has been resisted by power companies.

Coal, typically in the form of metallurgical coke, is also utilized in the steel-making industry, for example to reduce oxides of metals such as iron. In one known process, coal products are pelletized with water, silica, burned limestone and taconite, and are treated in a high temperature oven such as a cupola. To date, this method of generating metallic iron has received minimal attention.

What has been needed has been a more efficient method of energy production, utilizing, as the ultimate

source of fuel, coal and coal products. More particularly, what has been needed has been a method of energy production wherein values other than simply crude fuel values of the coal fuel are more efficiently and effectively utilized, for example in iron refining and boiler operation.

### OBJECTS OF THE INVENTION

Therefore, the objects of the present invention are: to provide a process for the generation of electrical power from coal fuel, wherein oil values in the coal are removed before the coal is utilized as a fuel; to provide such a method wherein following a liquefaction procedure a resultant coal char product is utilized in a reduction and melting process for the reduction of oxidized iron; to provide such a process wherein, during iron refining, hot product gases are formed which are utilized for the production of electricity, upon passage through a turbine arrangement; to provide such a process wherein the turbine arrangement preferably includes, in series, a gas turbine directly driven by gases from the iron refining process, and a steam powered generator, driven by steam produced in a boiler heated from a hot gas effluent from the gas turbines; to provide a process wherein steam generated in a boiler from hot effluent gases, from an iron refining process utilizing coal char, are in part utilized to provide a heat source for coal liquefaction in order to initially generate char material; to provide an overall process for the generation of oil products, the reduction of iron oxides, and the generation of electricity, which utilizes coal as the primary fuel source and source of reductant; and, to provide such a process which is relatively energy efficient, relatively simple to effect and which is particularly well-adapted for the proposed applications thereof. Other objects and advantages of the present invention will become apparent from the following descriptions, taken in connection with the accompanying drawings, wherein and set forth by way of illustration and example of various embodiments and applications of the present invention.

### SUMMARY OF THE INVENTION

The present invention concerns an overall process and plant design for the utilization of coal in an efficient process, wherein energy is produced and low cost iron refining is achieved. Further, potentially valuable oil products are extracted from the coal fuel source, and are made available for use in a variety of industries including the fuel industry, such as the diesel fuel industry. The overall process can be divided into a plurality of individual steps and stages; however, as will be understood from the detailed description, certain advantages are obtained from organization of the various stages into an efficient interdependent system, wherein energy from various stages is utilized in a relatively efficient manner to help drive other steps and stages. This will be readily apparent from the schematic representations described in detail below. The result is an overall useful plant construction, providing for oil generation, iron refining and energy production with relative cost efficiency.

During a first stage of the present invention, coal, provided as a fuel source, is treated in a liquefaction step, for the removal of volatile fractions therefrom. Simultaneously, undesired mineral values may also be extracted. An advantage to this latter, is that those mineral values which might otherwise interfere with de-

sired utilization of the coal as a fuel source are removed early in the process. Thus, a relatively low quality coal can be used in a process according to the present invention. As a result, cost efficiency and effectiveness are enhanced.

A variety of liquefaction procedures may be utilized during the liquefaction step. One method is solvent extraction followed by pyrolysis. Typically, a phenolic solvent would preferably be utilized, to initiate the extraction procedure. This would be followed by a relatively mild pyrolysis, using steam and oxygen, to drive off volatiles and remove additional valuable liquid fractions and generate a low volatile char product for use in the iron reduction procedure, i.e. the next stage.

Alternatives to the specific liquefaction procedure described above include: hot water treatment followed by water/steam extraction, rather than organic solvent extraction, and a mild pyrolysis; steam extraction only; and, pyrolysis only. The combination of organic solvent extraction and mild pyrolysis is generally preferred, for its energy efficiency and ability to achieve removal of substantially all relatively volatile components, leading to a particularly desired char for reduction purposes.

Char generated from a liquefaction step is usually fairly active, and is generally in a powdered form. Such material may spontaneously burn upon exposure to air, if dry. Thus, if it is to be stored for any considerable period of time, it is usually preferred that it be placed under an inert atmosphere and/or wetted down somewhat, typically about 30% moisture by weight being sufficient to inhibit combustion.

Generally, once formed the char material will be immediately prepared for utilization in an iron reduction and melting step. In one embodiment, this is preferably done through a pelletization process, wherein the char material is mixed with a binder, usually including lime and silica, and is treated with steam for induration, i.e. hardening into pellet form. The pellet form generally enhances the chemical reactions of iron reduction, and makes the char material easier to handle and less likely to be blown about by gases in the iron reduction step.

Char material formed during the First Stage described above, may be utilized for the reduction and melting of a variety of iron materials including iron ores such as taconite, and also scrap metal iron. If scrap metal iron is utilized, pellets made as described above are typically mixed directly with the scrap metal iron, and the refining process is run. If iron ore, such as taconite, is utilized, then preferably some of the char material is pelletized with the taconite itself, again the pellets including a binder.

In Stage Two, iron oxides are reduced typically in a smelter device such as an oven or cupola, in the presence of the char material which acts as a reductant. The products of a typical Stage Two generally include slag, liquid metal, and hot gases. The hot gases are utilized, directly and/or indirectly, to generate electrical power in the third general stage. In some embodiments Stage Two conditions may be varied slightly, for advantages. For example, chromite may be included in the pellets, to generate stainless iron. Also, kiln conditions may be used to form directly reduced iron.

In an alternate Stage Two embodiment, the coal char material is mixed with lime and is gasified. The coal gas is then brought into contact with iron material to be reduced and melted. In a preferred system, the coal char is gasified in a chamber such as a conventional

melter/gassifier. Iron material, such as ore, is fed into a separate chamber, wherein it is exposed to hot coal gas from the melter/gassifier. The reduced ore material is then fed directly into the melter/gassifier wherein it is melted, and drawn off as pig iron.

Stage Three involves utilization of the hot gas effluent from the cupola or reduction and melting process generally. In some embodiments, the cupola may be structured to operate under substantial pressures, to enhance efficiency and reduce residence time. In others, relatively low pressure processes may be used. In either case, the hot gases escaping from the reduction and melting process include generally about 30-40% carbon monoxide therein, among other gases. The rapidly cooling gases may be of relatively low temperature, 300°-600° F., in comparison to the cupola operating temperature, usually about 2,200°-2,600° F. (typically about 2,400° F.), and generally include particulate matter such as char dust therein. For a typical process, the escaping gases are passed through a filter arrangement or the like, for removal of the solid particulate manner.

In preferred Stage Three procedures, the waste gases are directed into a burner, wherein they are ignited in the presence of oxygen, to oxidize the carbon monoxide and increase the temperature of the gases considerably, typically to over 2,000° F. These very hot gases, having substantial energy, may then be driven into a gas turbine arrangement, whereat the energy of the gases is utilized directly for the generation of electricity. This is particularly desirable if the gases are under substantial pressure, as the gas turbine is an effective means of tapping the energy represented by the pressure. The cooler, lower energy, gases admitted from the gas turbine arrangement are then preferably directed into a boiler, for the generation of steam. Steam generated by the boiler may be utilized to drive a steam turbine, and produce electricity. Further, hot steam generated by the boiler may be utilized to facilitate many of the steps; for example as a heat source for the solvent and/or steam extraction/liquefaction of Stage One.

As the hot gases leave from the boiler, they still contain substantial heat which may be effectively utilized to facilitate processes according to the present invention. For example, these hot gases may be driven through a heat exchanger to heat air that is directed to various steps of the process, including air directed into the hot blast cupola in Stage Two, or any other Stage Two equipment.

In the schematic representations discussed in detail below, particularly efficient systems utilizing steam generated in a boiler, and heat generated from the reduction and melting steps, are shown. The drawings constitute a part of this specification, and include an exemplary embodiment of the invention, while illustrating various objects and features thereof. It will be recognized that the drawings, being schematic only, indicate general embodiments, and a variety of specific arrangements may be utilized according to the principles of the present invention.

#### BRIEF DESCRIPTION OF THE DRAWINGS

FIG. 1 is a schematic representation of a plant system for implementation of a process according to the present invention.

FIG. 2 is a schematic representation of a portion of a plant system according to an alternate embodiment of the present invention.

DETAILED DESCRIPTION OF THE  
PREFERRED AND ALTERNATE  
EMBODIMENTS

As required, detailed embodiments of the present invention are disclosed herein. However, it is to be understood that disclosed embodiments are merely exemplary of the invention which may be embodied in various forms. Specific structural and functional details disclosed herein are not to be interpreted as limiting, but rather as a basis for the claims and as a representative basis for teaching one skilled in the art to variously employ the present invention in virtually any appropriately detailed system.

In general, the process according to the present invention will be described in terms of three stages: a First Stage in which coal is treated for the formation of char and the removal of oil values; a Second Stage in which the char product is utilized in an iron-refining operation, to generate useful hot gases and reduced iron; and, a Third Stage in which hot gases from Stage Two are utilized in the generation of electricity. In a preferred arrangement as described and shown, the three stages are interacted, so that energy generated in each stage is effectively utilized throughout the entire process, in a preferred manner. This will become more apparent from the following descriptions.

STAGE ONE—PROCESSING OF THE COAL TO GENERATE CHAR AND COAL OIL PRODUCTS

Referring to FIG. 1, the reference numeral 1 generally designates Stage One of the process, wherein coal is treated to form char, with oil materials extracted therefrom. FIG. 1 will be understood to represent a power plant operated according to the principles of the present invention. At reference numeral 5, a coal feed is represented. A variety of grades of coal may be utilized in processes according to the present invention, in some instances including those grades which include too high a mineral content to generally be efficient as a conventional boiler feed stock.

In the First Stage, extraction/liquefaction procedures are employed to remove materials from the coal feed stock. A variety of methods are utilizable in processes according to the present invention. Generally, what is required is the ultimate removal of relatively volatile components and also extraction of mineral components, from the coal, to leave char material having relatively low volatiles content.

In a preferred application of the present invention, coal feed 5 is directed into a liquefaction system including an autoclave 6, whereat it is extracted by a solvent, such as a phenolic solvent or water/steam. Generally, extraction with a phenolic solvent at about 350° to 420° C., 450 psia, is effective to rapidly extract volatile materials out of coal. The hot solvent is represented fed into the autoclave via line 7, and is removed therefrom via line 8. The solvent, in FIG. 1, is shown at least partially heated by heat exchangers 10 and 11, described in further detail below. Heat exchanger 15 is positioned to cool the solvent from the extraction, directing same also through cooler 16 and into separator 17, wherein the extracted oil materials are separated from the solvent. The separator 17 may be of any of a variety of conventional types, including distillation systems, with the oil product being taken off at line 18 and the solvent being drawn off at line 19 and redirected into the autoclave 6, along line 7. For the embodiment shown the solvent, via

line 19, is directed through heat exchanger 15, as well as heat exchangers 10 and 11, so that it is heated sufficiently to generate the extraction via a continuous method. The volatiles removed via line 18 are shown separated into two components, at lines 20 and 21. Conventional separation techniques, not detailed, are generally utilized to separate more valuable coal oils, such as oils utilized as diesel fuel or the like, at line 20, with less valuable but readily burnable materials being directed via line 21 into a Stage Three boiler, described below, as a supplemental fuel source. Generally, at least about 65 gallons of useful oil can be extracted from a ton of coal.

At a second step in a preferred Stage One liquefaction system, the partially extracted residue from the autoclave 6 is directed into a pyrolysis oven or chamber 30, for mild pyrolysis, to ensure reduction of volatiles as far as reasonably possible. The reason for this is that it is desired to use a char with relatively little volatile material therein, in the iron reduction step of Stage Two. Typically, pyrolysis at about 600° C. and 1 atm., in the presence of steam and oxygen, readily extracts the remaining volatiles along line 31, leaving the char residue in a powder form. This relatively mild pyrolysis is advantageous, since it has relatively low energy demands, which can at least in part be met via heat supplied by heat exchanger 10. The volatiles drawn off via line 31 can be collected by conventional means, as desired. A steam circulation system, providing for a continual feed via line 32 from heat exchanger 10, can be provided in a conventional manner, if necessary or desired.

It will be understood that extractions and pyrolyses such as described may be used to remove metal salts from the char, as well as organic volatiles. Char material is shown being removed from pyrolysis oven 30, via line 35. Again this char material has a relatively low volatiles content, and is well suited for utilization in Stage Two as described below.

A variety of alternate liquefaction procedures may be utilized, including a two-stage liquefaction with hot water pretreatment and a water/steam extraction being utilized in place of the organic solvent. Generally, such a system would require a follow-up low temperature pyrolysis. The hot water pre-conditioning of the coal material facilitates extraction via the steam process. Such a process would typically involve, for example, pretreatment with water at about 200° C. for a brief period, typically 15–25 minutes, followed by steam extraction at about 375° C. and about 750 p.s.i.a. The follow-up pyrolysis would be as described above, in oven 30 for example at about 600° C. and atmospheric pressure.

Single step liquefaction processes may also be adaptable for utilization in association with systems according to the present invention, although generally such systems may be less efficient as they do not as readily lead to char having a very low volatiles content; or, when they do, they produce less of the valuable liquid products. In one type of single step system, only a pyrolysis process would be initiated, with the extraction process in the autoclave 6 being bypassed. In a second, only extraction in the autoclave 6 would be done, with a pyrolysis at 30 being bypassed. It will be understood that the liquefaction process chosen will generally depend upon cost, the nature of the coal feed, and the char product desired.

Regardless of the method of liquefaction chosen, the general process is to provide a low volatile char material for direction into Stage Two. In addition it is pre-

ferred to accomplish char generation in as low cost, energy efficient, method as possible. It will be readily understood that the solvent extraction/mild pyrolysis steps described in detail above will be generally advantageous as extreme conditions and long reaction times are generally avoided.

## STATE TWO—REDUCTION OF IRON MATERIAL

In Stage Two of a process according to the present invention, iron materials are reduced and/or melted to iron, for use in the manufacture of steel and the like. The iron material to be reduced and/or melted may be from a variety of sources, including iron ores and scrap metal iron. Generally, according to the present invention relatively expensive coke material is avoided and is replaced with a relatively low cost by-product of energy production, char, in a process for the manufacture of relatively inexpensive iron and steel products. This is accomplished, generally, as follows.

Char from takeoff 35 is generally in a powdered form, and is often highly reactive. If exposed, dry, to oxygen spontaneous combustion is possible and likely. Generally, rather than being stored the material is pulverized if necessary, and for preferred applications is formed into pellets for use in an iron reduction reaction.

The nature of the pellets formed will depend, in part, upon the nature of iron material to be reduced and/or melted. Generally a variety of iron sources may be utilized in processes according to the present invention. Most typically, two major sources will be used: oxides, for example in the form of iron ore, such as taconite; scrap metal iron; and, waste oxides, for example created during steel production and manufacturing process.

In FIG. 1, a process utilizing taconite is illustrated. The char material, after grinding in mill 40 is directed via line 41 into a mixing and pelletization system 42, wherein it is pelletized with various binder materials, and if necessary the iron ore. A variety of conventional pellet forming mechanisms such as mixer-mullers and pelletizing discs may be utilized as part of system 42. Generally, what is required is that the char material be mixed with ore, shown introduced via line 45, in a manner ensuring pellet formation. To accomplish pellet formation, binder materials such as water, silica and burned limestone are added, in small amounts, to the pellets. In FIG. 1, water, silica and limestone are shown fed via lines 46, 47 and 48, respectively. These materials enhance agglomeration, under application of heat.

Typically, pelletization includes formation of a plurality of small pellets, about 4-1½ inches in diameter, each including, by weight, about 10-18% char, about 60-80% taconite, about 8-15% water, and about 1-8% burned lime, although variations may be used. Such pellets are generally readily agglomerated and provide sufficient association of the carbon (char) with the iron, to facilitate the reduction process when heat is applied.

Agglomeration is generally facilitated by application of heat and steam. Referring to FIG. 1, the pellets 50 formed by pellet maker 42 are shown directed via line 51 into autoclave 52 for induration. In autoclave 52, heat and steam are applied, to provide for a stable, hard, pellet material. Typically, steam at about 175°-225° C., under pressures of 75-300 psi may effectively be utilized to generate the hard particles. It will be understood, however, that a variety of pressure and temperature conditions may be utilized, depending upon the specific pellet composition involved, and the pellet use in-

tended. Further, optimization of temperature and pressure may be found empirically for various systems, to enhance energy savings and achieve a desired induration time.

5 Pellets, such as those previously described, may be directed into an oven such as a cupola, for reduction of the iron. In some instances, however, rather than taconite or iron ore, scrap metal iron may be utilized. Under such circumstances, generally the pellets of char material should be formed without the iron mixed directly therein, but rather only from char material containing enough silica, limestone and/or water to provide efficient agglomeration. For this latter modification of the process, generally the char pellets would be charged 10 into the cupola, as a mixture with scrap metal iron.

15 Referring to FIG. 1, since the induration in autoclave 52 is a relatively low temperature process, it may be accomplished at least in part using steam fed from line 55, and heated via heat exchanger 56. The preferred 20 heat exchanger 56, is shown at least in part heated via steam lines 57 and 58, from the boiler of Stage Three. This will be described in further detail below. A result of this advantage is a lower energy-consuming overall process.

25 Pellets from autoclave 52 are shown, in FIG. 1, being directed into cupola 60 via line 61. A variety of conventional cupolas 60 may be utilized in processes according to the present invention. Further, it is foreseen that in some applications cupolas modified for operation at a relatively high pressures, for example 100-200 psia, may be used to facilitate the reduction process, and to enhance later energy production, in manners to be described below. Other oven systems, such as kilns, may be used in some processes.

30 Generally, feed stock for the cupola 60 is fed in as a solid, piled such that air or the like can pass therethrough. If taconite is to be reduced, typically the iron-ore containing pellets are simply piled into the cupola or furnace. On the other hand, if scrap metal iron is involved, char pellets are mixed into a pile in the furnace, along with the scrap metal. Hot air, used to facilitate the reduction process, is shown fed into the hot cupola 60 via line 67. Slag and molten metal are shown removed via line 68. It will be readily understood that this process comprises a relatively low cost, energy efficient, step in the manufacture of steel products or the like. Further, relatively low capital costs are involved, since high efficiency permits relatively small smelters or cupolas to be used. The low capital costs are also enhanced by the valuable oil extraction of Stage One, and the relatively efficient energy generation of Stage Three.

35 Hot gases escaping from the cupola 60 are shown drawn off at line 75. From a typical cupola operation these hot gases include about 30-40% carbon monoxide, and are at a temperature of about 300°-600° F. In a typical cupola operation, the gas blown into the cupola 60 is preferably around 800°-1,200° F., and in the cupola 60 it is heated to about 2,500°-2,800° F. The gases are generally rapidly cooling as they transfer heat energy to the materials in the cupola 60. In some systems according to the present invention, as indicated above, the cupola 60 may be operated under substantial pressures, on the order of about 125-175 psi. In other instances, pressures near atmospheric may be utilized.

40 The gases drawn off through line 75 are utilized in Stage Three (reference numeral 76) in a preferred manner, to generate electrical power.

### STAGE THREE—ELECTRICAL POWER GENERATION

In Stage Three, as indicated above, the hot gases removed from the cupola 60 are utilized to generate electrical power. Further, heat from these gases is utilized, as described below, to facilitate the other stages of the process. Referring to FIG. 1, hot gases from the cupola 60, via line 75, are preferably directed through a filter or cleaner 80, for the removal of particulate material entrapped therein, from the cupula process. Such materials include, for example, products from hot gas treatment of the char pellets. This screen or filter process generally is used to protect downstream equipment from injury. Sulfur may also be removed very effectively at this point, with an absorbent, for example in the gas screen.

As previously indicated, the gas in line 75 includes a substantial amount of carbon monoxide (generally 30–40%) therein. Advantage may be taken of this carbon monoxide content. In particular, the carbon monoxide is oxidized with air, at burner 81. This increases the temperature of the gas to near 1800°–2200° F., and further leads to the destruction of the potentially hazardous carbon monoxide. Air for the oxidation is shown fed into burner 81 via line 82. Hot, oxidized, gas is shown drawn off at line 83.

The high temperature gases from burner 81 are used for the generation of electricity. It will be readily understood that there are advantages to the utilization of gas under substantial pressure from the cupola 60, as more efficient turbine operation can be achieved. For preferred plant systems, gas turbine 85 provides for energy production, from cupola gases.

After passing through the gas turbine 85, the hot gases, illustrated by line 86, in preferred processes will still represent a substantial energy source, due to their still relatively high temperature, typically about 800°–1,000° F. These waste gases are shown directed into boiler 90, for the generation of steam. The steam may be utilized in a variety of manners. For example:

Steam line 91 is shown being used to drive turbine 92, for the production of still more electricity. The outlet steamline 95, from turbine 92, is shown providing heat to heat exchanger 11, which is utilized to drive the original extraction in Stage One. Also, outlet line 95 is shown communicating with heat exchanger 56, via lines 57 and 58, to provide an energy source for induration of pellets in Stage Two. Ultimately, steam or water is returned to boiler 90, via line 96.

Very hot steam, on the order of 400° C. or higher, is shown being drawn off of boiler 90, via line 105. This steam is directed via line 105 into heat exchanger 10, to facilitate the original extraction process and also the pyrolysis process. Once cooled, this steam/water is returned to the boiler via line 106.

Heat feed to the boiler 90 may be from a variety of systems. For the preferred system according to the present invention, the majority of the heat drive is provided via the hot gases drawn off of the cupola 60, indicated in line 86. Other sources of heat include energy derived from the less important and less valuable coal oil products, shown directed into boiler 90 via line 21.

Hot gases escaping from the boiler 90 are shown drawn off at line 110. Such gases are still relatively hot, and can be utilized in heat exchanger 111 for a variety of purposes, including to heat air used in boiler 90, shown

introduced via line 112, and also to help heat air directed into the cupola, shown in line 67. Ultimately, the gases from line 110 are discharged to the atmosphere, as indicated in line 113. Typically, they first pass through a scrubber arrangement or the like, not shown, which may be of a conventional construction and is used for pollution control. While the gases include substantial amounts of carbon dioxide, overall emissions may be lower than for conventional systems wherein less efficient use of the coal is made.

From the above descriptions it is readily understandable that an advantage to the present invention is that an overall interdependent system is provided, wherein coal is very efficiently utilized in a combination energy generation and iron refining facility. Relatively highly valuable components in the coal, i.e. the coal oils, are originally extracted. A formerly low value char material is utilized both to reduce iron, and lessen the costs of iron and steel production, and to produce a gas product facilitating efficient energy generation.

### ALTERNATE STAGE TWO OPERATION

In an alternate Stage Two operation, a pelletization procedure is avoided. Referring to FIG. 2, the coal char from Stage One is fed into pressurized feed bin 200 via line 201, wherein it is mixed with lime, fed via line 202. This mixture is fed under pressure into a conventional melter/gassifier 205, via line 206. In melter/gassifier 205 sufficient heat is provided to gassify the coal char. Off gases are fed via line 210 into a reduction furnace which includes therein oxidized iron material such as ore, fed via line 211. The off gases from the reduction are removed via line 212, and are used analogously to off gases from a cupola as previously described. For a typical system, the reduced iron material is fed via line 215 directly into the melter/gassifier wherein it is melted and removed via line 216.

A typical process according to the present invention will be understood from the following proposed example.

### EXAMPLE 1

The following provides a description of operation of a typical processing plant, on a scale which would generally be useful, according to the present invention. It will be understood that a variety of plant sizes, and operating conditions, may be utilized according to the principles described previously. For the example illustrated, it is envisioned that coal feed into the system will be on the order of about 79 tons per hour. From the extraction and pyrolysis, for a typical coal feed, about 31 tons per hour of oils and 21 tons per hour of volatile gases, can be released, resulting in formation of about 27 tons of char per hour.

Pelletization depends upon the nature of the iron to be reduced. If iron ore such as taconite is involved, about 13 tons per hour of the 27 tons per hour of the char should be hardened into pellets without the taconite, via steam induration as previously described, with sufficient water and lime being provided to facilitate pellet integrity. About 14 tons per hour of the char should be mixed with about 70 tons per hour of the iron ore, 4.5 tons per hour of lime, and 11.5 tons per hour of water, to form about 100 tons per hour of pellets. Typically, along with the steam induration process, a drying step may be utilized to drive moisture out of the pellets, resulting in about 90 tons per hour of ore-containing pellets being fed into the cupola, with the cupola also

being fed with the 13 tons per hour of char which was pelletized without ore.

As previously indicated, the cupola can be operated under a variety of conditions. For a typical run, about 116 tons per hour of combustion air should be driven 5 into the cupola, to form about 161 tons per hour of off-gases, 18 tons per hour slag, and 40 tons per hour of reduced iron, i.e. pig iron.

As previously described, the gases in the cupola are rapidly cooling, as they pass through the material in the 10 cupola. However, these gases are reheated during the burning process, to a relatively high temperature. This permits efficient energy generation via the gas turbine, and the follow-up boiler/steam system. Generally, conventional equipment can be utilized to accomplish this. 15

It is to be understood that while certain embodiments of the present invention have been illustrated and described, the invention is not to be limited to the specific arrangements described herein, except as provided for by the following claims.

What is claimed and desired to be secured by Letters Patented is as follows:

1. A process for the production of electricity; said process including the steps of:

- (a) providing a low grade coal fuel;
- (b) performing a pyrolysis procedure on the coal fuel at a temperature of about 600° C. to remove oil and volatiles therefrom, and to generate a resultant coal char product;
- (c) pelletizing the coal char product to form coal char product pellets, said step of pelletizing comprising pelletizing at least a portion of the coal char product in combination with reducible solid iron material to form coal char pellets containing reducible solid iron material;
- (d) charging a cupola with the coal char product and the reducible solid iron material, said step of charging a cupola being characterized by charging substantially all the coal char product in the form of coal char product pellets and substantially all the 40

reducible solid iron material in the form of pellets containing the coal char product in combination with the reducible solid iron material;

- (e) reducing and melting all the reducible solid iron material in the coal char pellets by heating the pellets in the cupola at a suitable temperature under a pressure of at least about 100 psi in the presence of a sufficient upward flow of process gases, with the resultant formation of hot product gases;
- (f) tapping the hot product gases from an upper portion of the cupola;
- (g) directing the hot product gases downstream to electrical production equipment; and
- (h) producing electricity from the hot product gases.

2. The process according to claim 1 wherein said step of reducing and melting the reducible solid iron material is conducted at a temperature of at least about 2,400° F.

20 3. The process according to claim 2 wherein said step of reducing and melting the reducible solid iron material at a temperature of at least about 2,400° F. is conducted at a pressure of at least about 125 psia.

25 4. The process according to claim 1 wherein said step of producing electricity from the hot product gases includes passing the hot product gases through a gas turbine to generate electrical power and then through a boiler to generate steam; at least a portion of the steam being utilized to drive a turbine and generate electrical power.

5. The process according to claim 1 wherein said step of pelletizing the coal char product includes mixing the coal char product with a binder selected from the group consisting of burned lime, silica, water, and mixtures 35 thereof to form pellets.

6. The process according to claim 1 further including utilizing heat derived from the hot product gases in the performance of steps (b) and (e) to achieve a thermally efficient process.

\* \* \* \* \*

UNITED STATES PATENT AND TRADEMARK OFFICE  
CERTIFICATE OF CORRECTION

PATENT NO. : 5,055,131  
DATED : October 8, 1991  
INVENTOR(S) : John M. Lehto

It is certified that error appears in the above-identified patent and that said Letters Patent is hereby corrected as shown below:

Column 6, line 41, "pace" should read --place--.

Column 6, line 68, "is'" should read --is--.

Column 8, lines 37-38, "iro-nore" should read  
--iron ore--.

Column 12, line 7 (claim 1(e)), "psi" should read  
--psia--.

Signed and Sealed this  
Twelfth Day of April, 1994

Attest:



BRUCE LEHMAN

Attesting Officer

Commissioner of Patents and Trademarks